

# UNITED STATES PATENT OFFICE.

JOHN M. FERRY, OF BALTIMORE, MARYLAND.

## COMPOUND FOR WATER-TIGHT JOINTS.

1,153,427.

Specification of Letters Patent. Patented Sept. 14, 1915.

No Drawing.

Application filed September 8, 1914. Serial No. 860,566.

*To all whom it may concern:*

Be it known that I, JOHN M. FERRY, a citizen of the United States, residing at Baltimore, in the State of Maryland, have 5 invented certain new and useful Compounds for Water-Tight Joints, of which the following is a specification.

My composition consists of the following ingredients, combined in the proportions 10 stated, viz:

|        |              |
|--------|--------------|
| Sulfur | 30 per cent. |
| Loam   | 40 per cent. |
| Tar    | 30 per cent. |

15 These ingredients are to be thoroughly mingled by heating same. After the ingredients have been thoroughly mixed the composition is poured into barrels, tanks, or other suitable vessels, and allowed to 20 harden.

Copies of this patent may be obtained for five cents each, by addressing the "Commissioner of Patents, Washington, D. C."

In using the composition it is only necessary to heat same until it flows and then pour into the joints and allowed to harden, whereby a water-tight and air-tight joint will be formed.

25

I claim:

The herein-described composition of matter for forming water-tight joints, consisting of sulfur thirty per cent., loam forty per cent. and tar thirty per cent., substantially as described.

30 In testimony whereof I affix my signature in presence of two witnesses.

JOHN M. FERRY.

Witnesses:

CHAPIN A. FERGUSON,  
CHARLES E. GARITEE.